

1

3,495,981

## COLOR DEVELOPING PROCESS

Tadashi Nagae and Haruhiko Iwano, Ashigara-Kamigun, Kanagawa, Japan, assignors to Fuji Sashin Film Kabushiki Kaisha, Ashigara-Kamigun, Kanagawa, Japan, a corporation of Japan  
No Drawing. Filed June 15, 1966, Ser. No. 557,638  
Claims priority, application Japan, June 17, 1965,  
40/36,165

Int. Cl. G03c 7/30, 5/30

U.S. Cl. 96—55

4 Claims 10

## ABSTRACT OF THE DISCLOSURE

Exposed silver halide color photographic elements are developed with a color developer containing p-phenylenediamine or derivative thereof, polyoxyethylene alkylphenyl ether and p-aminophenol or derivative thereof, whereby the color developing speed is promoted, the deficiency in silver bleaching and color contamination are reduced, and the photographic qualities are improved.

The present invention relates generally to an improved color developing process for silver halide color photographic elements and more particularly to a color developing process using polyoxyethylene alkylphenyl ether and p-aminophenol or derivatives thereof to promote the color developing speed, reduce the deficiency in silver bleaching and color contamination, and to improve picture qualities.

Since a conventional color developer containing as a color developing agent p-phenylenediamine or derivatives thereof is low in developing power as compared with a general black and white developer, the pH value of the processing solution must be extremely high or the developing procedure must be conducted for a very long period of time. Accordingly, there have hitherto been employed various color developing accelerators but the use of such conventional color developing accelerators frequently causes at development fogging at the unexposed areas resulting in contaminating the pictures or images and further, if the developing period of time is reduced for preventing the formation of fog, no increase in the color density of the image portions is observed and hence the color developing processing cannot be conducted effectively.

In particular, in a color developing process using a color developer containing couplers therein, the use of a color developing accelerator frequently causes undesirable color fogging or color contamination.

Further, the presence of the developing accelerator in a bleaching process for developed silver after the color development frequently reduces the oxidation speed of silver, that is, causes the phenomenon of so-called insufficient silver bleaching.

Thus, there are presently very few color development accelerators having excellent properties as aforementioned.

Accordingly, an object of the present invention is to accelerate the color developing speed and also increase the color density.

Another object of the present invention is to improve the silver-bleaching in color photographic processing.

Still another object of the present invention is to reduce or prevent the decontamination or color contamination in color photography.

It has been found that after investigation that by using a color developer containing p-phenylenediamine or derivatives thereof incorporated with a below-stating polyoxyethylene alkylphenyl ether and p-aminophenol or a derivative thereof, the color developing speed can be re-

2

markably increased as well as the silver bleaching improved and hence decontamination or color decontamination reduced to improve the qualities of photographic pictures.

It is known that the use of a polyoxyethylene alkylphenyl ether alone accelerates the developing speed but at the same time results in undesirable contamination or color contamination. Further, some kinds of couplers are present at color development, the use of such a developing accelerator will cause insufficient silver bleaching. However, if the developing accelerator is used together with p-aminophenol or derivatives thereof in color development, the developing speed is accelerated more effectively, as compared with the case of using the developing acceleration alone, and the abovementioned various faults are reduced.

The polyoxyethylene alkyl phenyl ether used in the present invention can be represented by the following general formula



wherein R and R' are a hydrogen atom or an alkyl group having 1 to 5 carbon atoms and n is a number of 5 to 50.

The compounds shown by the above general formula are illustrated as follows:



The suitable amount of the abovementioned polyoxyethylene alkylphenol ether is usually from 0.5 to 10 g./

er. The amount may be less or more than the range if it is less than 0.5 g./liter the effect of the addition thereof will be weak and if higher than 10 g./liter the effect will not be increased more and hence the addition of too much amount of the compound is unnecessary.

The p-aminophenol derivatives used in this invention are N-methylaminophenol sulfate (metol), o,p-diaminophenol hydrochloride (amidol), and N-benzyl-p-aminophenol. Although the effect may be slightly less than those of the abovementioned derivatives, p-aminophenol may be so used in this invention. In this respect, it must be understood that the use of p-aminophenol or the derivatives thereof among various black and white developing agents is important in this invention since the use of other black and white developing agents together with the abovementioned developing accelerator increases, on the contrary, the contamination or color contamination. Further, if the abovementioned p-aminophenol or the derivatives thereof are added alone in a color developer, a black and white development occurs simultaneously with the occurrence of a color development, which results in the reduction of color density and only if the amount thereof is properly selected some extent of the increase in color density is observed in a limited range of exposure and developing period of time. However, as the abovementioned polyoxyethylene alkylphenyl ether is present together with the p-aminophenol derivatives or p-aminophenol in the color developer, the color density can be remarkably increased without increasing color fogging.

A suitable amount of p-aminophenol or the derivatives thereof to be incorporated in the developer is 0.1 to 1 g./liter. The amount may be less or higher than this range but if the amount is less than 0.1 g./liter, the effect of addition thereof becomes insufficient and if it is higher than 1 g./liter the color density tends to decrease on the contrary. Two or more kinds of the abovementioned p-aminophenol and the derivatives thereof may be used in this invention.

Thus, by using the abovementioned two compounds according to the present invention, said two compounds being impracticable individually owing to their drawbacks, the faults of the two compounds are compensated for by each other to make possible the practical use thereof as well as an unexpected remarkable development accelerating effect which has never been expected from the interaction of them.

The present invention may generally be applied to color photographic elements using a color developer containing p-phenylene-diamine or derivatives thereof, such as negative color photographic films, photographic color papers, photographic color reversal films and the like. In particular, the most effective results of this invention can be obtained in the case of conducting this invention about a yellow color developer for photographic color reversal film having technical difficulties in silver bleaching and color decontamination.

The following examples illustrate but do not limit the present invention:

#### EXAMPLE 1

A test sample which had been prepared by applying a blue-sensitive gelatino silver bromo-iodide emulsion to cellulose acetate film was exposed by means of a sensitometer and subjected to the following processings:

first development ..... min. at 27° C. 3  
water rinsing ..... min. 4  
reversal exposure (tungsten lamp) ..... CMS 200  
color development ..... min. 5  
water rinsing ..... min. 4  
leaching ..... min. 2  
water rinsing ..... min. 1  
fixing ..... min. 2  
water rinsing ..... min. 2

The compositions of the processing baths were as follows:

|    |                                                                         |
|----|-------------------------------------------------------------------------|
| 5  | First developer:                                                        |
|    | N-methyl-p-aminophenol sulfate ..... g. 2.0                             |
|    | Sodium sulfite ..... g. 90.0                                            |
|    | Hydroquinone ..... g. 8.0                                               |
| 10 | Sodium carbonate (monohydrate) ..... g. 52.5                            |
|    | Potassium bromide ..... g. 5.0                                          |
|    | Potassium thiocyanate ..... g. 100                                      |
|    | Water to make 1 liter.                                                  |
| 15 | Color developer:                                                        |
|    | Sodium sulfite ..... g. 5.0                                             |
|    | p-Amino-N,N-diethylaniline sulfite ..... g. 2.5                         |
|    | Potassium bromide ..... g. 1.0                                          |
| 20 | Potassium iodide (0.1% aq. soln.) ..... ml. 5                           |
|    | 1 - w - benzoyl - 4 - (p - toluenesulfonamido)-acetanilide ..... g. 1.2 |
|    | Sodium hydroxide ..... g. 2.5                                           |
|    | Water to make 1 liter.                                                  |
| 25 | Bleaching solution:                                                     |
|    | Potassium ferricyanide ..... g. 100                                     |
|    | Potassium bromide ..... g. 10                                           |
|    | Borax ..... g. 2                                                        |
| 30 | Boric acid ..... g. 1                                                   |
|    | Water to make 1 liter.                                                  |
| 35 | Fixing solution:                                                        |
|    | Sodium thiosulfate ..... g. 150                                         |
|    | Sodium sulfite ..... g. 10                                              |
|    | Water to make 1 liter.                                                  |

The color densities and the silver-bleaching effects were measured in this processing about the cases of using the polyoxyethylene alkylphenyl ether or the p-aminophenol derivative alone and using both of them, the results of which are shown in Table 1. The color density is shown by the value obtained by measuring the maximum density range of thus processed film using a blue filter light and the silver-bleaching effect is shown by the value of the blackened density ( $D_R$ ) caused by the remaining silver measured by using a red filter light divided by the color density value ( $D_B$ ) obtained from measuring by using a blue filter light.

TABLE 1

| 55 | Compound Added in Color Developer, g./liter |                   | Color Density, $D_B$ Max. | Silver Bleaching Effect ( $D_R/D_B$ ) |
|----|---------------------------------------------|-------------------|---------------------------|---------------------------------------|
|    | Compound D                                  | Benzylaminophenol |                           |                                       |
|    | 0                                           | 0                 | 2.4                       | 0.185                                 |
|    | 1.0                                         | 0                 | 2.8                       | 0.200                                 |
|    | 0                                           | 0.2               | 2.4                       | 0.165                                 |
|    | 1.0                                         | 0.2               | 2.9                       | 0.165                                 |

Thus, a yellow color image having a high color density and a high transparency was obtained by using compound (D) and benzylaminophenol together as compared with the cases of using compound (D) or benzylaminophenol individually.

#### EXAMPLE 2

70 To a cellulose acetate film were applied a red-sensitive gelatino silver bromo-iodide emulsion, a green-sensitive gelatino silver bromo-iodide emulsion, a yellow filter layer composed of colloidal silver for absorbing blue light, and a blue-sensitive silver bromo-iodide emulsion in this order to provide a multi-layered color photographic film,

which was exposed using a sensitometer and subjected to the following processings:

|                                    |                |      |
|------------------------------------|----------------|------|
| First development                  | min. at 27° C. | 4    |
| Water rinsing                      | min            | 4    |
| Reversal red exposure              | CMS            | 100  |
| Cyan color development             | min            | 5    |
| Water rinsing                      | min            | 2    |
| Reversal blue exposure             | CMS            | 200  |
| Yellow color development           | min            | 5    |
| Water rinsing                      | min            | 2    |
| Second black and white development | min            | 2    |
| Water rinsing                      | min            | 2    |
| Reversal white exposure            | CMS            | 2000 |
| Magenta color development          | min            | 5    |
| Water rinsing                      | min            | 4    |
| Bleaching                          | min            | 2    |
| Water rinsing                      | min            | 1    |
| Fixing                             | min            | 2    |
| Water rinsing                      | min            | 2    |

The compositions of the processing solutions are as follows:

The compositions of the first developer and the second black and white developer are same as the composition of the primary developing solution in Example 1.

#### Cyan color developer:

|                                                    |    |      |
|----------------------------------------------------|----|------|
| Sodium sulfite                                     | g  | 5.0  |
| 4-amino-3-methyl-N, N-diethylaniline hydrochloride | g  | 1.5  |
| Sodium carbonate (mono-hydrate)                    | g  | 15.0 |
| Potassium bromide                                  | g  | 1.0  |
| Potassium iodide (0.1% aq. soln.)                  | ml | 2    |
| 1,5-dihydroxy-2-6-dibromonaphthalene               | g  | 1.2  |
| Sodium hydroxide                                   | g  | 2.0  |
| Water to make 1 liter.                             |    |      |

The composition of the yellow developer is same as that of the color developer in Example 1.

#### Magenta color developer:

|                                                       |    |     |
|-------------------------------------------------------|----|-----|
| Sodium sulfite                                        | g  | 5.0 |
| 4-amino-3-methyl-N, N-diethylaniline hydrochloride    | g  | 2.0 |
| Potassium bromide                                     | g  | 0.2 |
| 1 - phenyl - 3 - (m - nitrobenzoylamino)-5-pyrazolone | g  | 1.4 |
| Sodium hydroxide                                      | g  | 2.5 |
| n-Butylamine                                          | ml | 5   |
| Water to make 1 liter.                                |    |     |

The compositions of the bleaching solution and the fixing solution are same as those in Example 1.

The effect of the addition of the compounds of this invention to the yellow color developer in the above processings is shown in Table 2. In the table, the color density ( $D_B$ ) was measured by a blue filter light. The silver bleaching was measured about the samples exposed to yellow patch. The color contamination (1) shows the ratio of the color density ( $D_G$ ) obtained by measuring with a green filter light a sample exposed to yellow patch to the color density ( $D_B$ ) obtained by measuring it with a blue filter light, that is, the ratio of unnecessary magenta color components in the yellow image and the color contamination (2) shows the ratio of the color density ( $D_B$ ) obtained by measuring with a blue filter light a sample exposed to a magenta patch to the color density ( $D_G$ ) obtained by measuring it with a green filter light, that is, the ratio of unnecessary yellow components in the magenta color image.

TABLE 2

| Addition Compounds | Color Density ( $D_B$ ) | Silver Bleaching Effect ( $D_B/D_B$ ) | Color Contamination |                   |
|--------------------|-------------------------|---------------------------------------|---------------------|-------------------|
|                    |                         |                                       | (1) ( $D_G/D_B$ )   | (2) ( $D_B/D_G$ ) |
| Compound E         |                         |                                       |                     |                   |
| Metol              |                         |                                       |                     |                   |
| 5                  |                         |                                       |                     |                   |
| 0                  | 0                       | 3.0                                   | 0.13                | 0.83              |
| 1.0                | 0                       | 3.3                                   | 0.20                | 0.38              |
| 0                  | 0.2                     | 3.15                                  | 0.08                | 0.44              |
| 1.0                | 0.2                     | 3.6                                   | 0.11                | 0.42              |
| 2.0                | 0.3                     | 3.65                                  | 0.11                | 0.40              |
| 10                 |                         |                                       |                     |                   |

## EXAMPLE 3

By repeating the procedure as in Example 2 using a standard composition for the yellow developer while incorporating the compounds of this invention in the cyan color developer, the results of which are shown in Table 3.

TABLE 3

| Addition Compound | Coupling Density ( $D_R$ ) | Color Contamination |                   |
|-------------------|----------------------------|---------------------|-------------------|
|                   |                            | (1) ( $D_B/D_R$ )   | (2) ( $D_R/D_B$ ) |
| Compound B        |                            |                     |                   |
| Amidol            |                            |                     |                   |
| 20                |                            |                     |                   |
| 0                 | 0                          | 3.0                 | 0.41              |
| 1.0               | 0                          | 3.35                | 0.33              |
| 0                 | 0.03                       | 2.9                 | 0.30              |
| 1.0               | 0.03                       | 3.4                 | 0.27              |
| 21                |                            |                     |                   |

The color density in Table 3 is a value measured by using a red filter light, the color contamination (1) shows the unnecessary yellow components in the cyan color patch and the color bleaching (2) shows the unnecessary cyan color components in yellow patch.

## EXAMPLE 4

A gelatino silver bromo-iodide emulsion containing a yellow coupler was applied to a cellulose acetate film to provide a test sample, which was exposed by means of a NSG actionometer and then subjected to the following processings:

|    |                   |                |    |
|----|-------------------|----------------|----|
| 40 | Color development | min. at 24° C. | 8  |
|    | Water rinsing     | sec            | 30 |
|    | Primary fixing    | min            | 4  |
|    | Water rinsing     | min            | 5  |
|    | Bleaching         | min            | 4  |
|    | Water rinsing     | min            | 5  |
|    | Secondary fixing  | min            | 4  |
|    | Water rinsing     | min            | 5  |

The compositions of the processing solutions were as follows:

|    |                                                                  |    |     |
|----|------------------------------------------------------------------|----|-----|
| 50 | Color developer:                                                 |    |     |
|    | Benzyl alcohol                                                   | ml | 3   |
|    | Hydroxylamine sulfate                                            | g  | 2   |
|    | Sodium sulfite                                                   | g  | 2   |
|    | 3-methyl-4-amino-N-ethyl-methanesulfonamido-ethylaniline sulfate | g  | 1.5 |
|    | Sodium carbonate (mono-hydrate)                                  | g  | 60  |
|    | Potassium bromide                                                | g  | 1   |
|    | Sodium hydroxide                                                 | g  | 0.1 |
|    | Water to make 1 liter.                                           |    |     |

## Fixing solution (first):

|    |                        |    |     |
|----|------------------------|----|-----|
| 65 | Sodium sulfite         | g  | 15  |
|    | Sodium thiosulfate     | g  | 150 |
|    | Acetic acid (28%)      | ml | 48  |
|    | Boric acid             | g  | 7   |
|    | Potassium alum         | g  | 15  |
|    | Water to make 1 liter. |    |     |

## Bleaching solution:

|    |                        |   |    |
|----|------------------------|---|----|
| 70 | Potassium bromide      | g | 20 |
|    | Potassium dichromate   | g | 5  |
|    | Potassium alum         | g | 40 |
|    | Sodium acetate         | g | 8  |
|    | Acetic acid            | g | 57 |
|    | Water to make 1 liter. |   |    |

ixing solution (second):

|                        |       |     |     |
|------------------------|-------|-----|-----|
| Sodium thiosulfate     | ----- | g-- | 150 |
| Sodium sulfate         | ----- | g-- | 15  |
| Potassium alum         | ----- | g-- | 15  |
| Water to make 1 liter. |       |     |     |

The results of incorporating the compounds of this invention in the color developer in the above processings are shown in Table 4.

TABLE 4

| Addition Compound | Compound F | Metol | Color Density (D <sub>B</sub> ) | Relative Sensitivity | Silver Bleaching Effect           |           |
|-------------------|------------|-------|---------------------------------|----------------------|-----------------------------------|-----------|
|                   |            |       |                                 |                      | (D <sub>R</sub> /D <sub>B</sub> ) | Color Fog |
|                   | 0          | 0     | 1.50                            | 2.10                 | 0.15                              | 0.26      |
|                   | 1.0        | 0     | 1.65                            | 2.20                 | 0.20                              | 0.30      |
|                   | 0          | 0.2   | 1.48                            | 2.10                 | 0.12                              | 0.23      |
|                   | 1.0        | 0.2   | 1.69                            | 2.24                 | 0.12                              | 0.22      |

(In the table, the relative sensitivity was shown by the relative value of the logarithmic exposure amount at the point where the density reaches fog +0.2.)

## EXAMPLE 5

By repeating the sample procedure as in Example 1 using .15/liter of methylaminophenol sulfate instead of benzyl aminophenol and 2.0 g./liter of compound (K) instead of compound (D), the following results were obtained:

TABLE 5

| Addition Compound | Compound K | Methylaminophenol | Color Density (D <sub>B</sub> /Max.) | Silver Bleaching Effect           |       |
|-------------------|------------|-------------------|--------------------------------------|-----------------------------------|-------|
|                   |            |                   |                                      | (D <sub>R</sub> /D <sub>B</sub> ) |       |
|                   | 0          | 0                 | 0                                    | 2.4                               | 0.185 |
|                   | 2.0        | 0                 | 0                                    | 2.7                               | 9.200 |
|                   | 0          | 0.15              | 0.15                                 | 2.4                               | 0.170 |
|                   | 2.0        | 0.15              | 0.15                                 | 2.8                               | 0.170 |

We claim:

1. In color developing process for color photographic silver halide elements, a color developer containing a member selected from the group consisting of p-phenylenediamine and the derivatives thereof is used, the improvement which comprises in said color developer (A) phenyl ether represented by the general formula:



wherein R and R' represent a member selected from the group consisting of a hydrogen atom and an alkyl group having 1 to 5 carbon atoms and n is a number of from 5 to 50, and (B) at least one component selected from the group consisting of N-methyl-p-aminophenol, o,p-diaminophenol, N-benzyl-p-aminophenol and p-aminophenol.

2. The color developing process as in claim 1, wherein the amount of said component (B) to the color developer is 0.1 to 1 g./liter.

3. The color developing process as in claim 1, wherein the amount of said component (A) to the color developing solution is 0.5 to 10 g./liter.

4. The color developing process as in claim 1, wherein at least one of the R and R' groups of component A is an alkyl group.

## References Cited

## UNITED STATES PATENTS

- 2,531,832 11/1950 Stanton ----- 96—66.3  
 3,158,483 11/1964 Lowe et al. ----- 96—66.3  
 3,300,305 1/1967 Pesch et al. ----- 96—22

35 J. TRAVIS BROWN, Primary Examiner

U.S. Cl. X.R.

96—66.3